

## UNITED STATES PATENT OFFICE

JOSEPH C. WASSON, OF PITTSBURGH, PENNSYLVANIA, ASSIGNOR TO PENNSYLVANIA LUBRICATING COMPANY, A CORPORATION OF DELAWARE

## HOT-JOINT COMPOUND

No Drawing.

Application filed February 1, 1927. Serial No. 165,249.

This invention relates to sealing compounds having lubricating properties, as for example joint sealing compounds, and comprises an improved composition of matter particularly adapted for use as a pipe thread or hot joint compound. The nature of this material will be fully understood in regard to both its manufacture and use from the following description.

10 Pipe thread or hot joint compounds have been widely used in the past and while these compounds often produce a tight joint, there is great difficulty in breaking the joint, and the threads or other surfaces are consequently often damaged. My improved compound has the valuable property of retaining almost indefinitely its sealing and lubricating qualities so that joints may be taken down with the greatest ease after long periods of severe service and with no damage to the contacting surfaces.

I have found that the metallic salts of the sulfonic acids are valuable ingredients for hot joint compounds. These sulfonic acids are made by extracting the oily layer resulting from the treatment of hydrocarbon oil with concentrated or fuming sulfuric acid with an organic solvent such as alcohol. The salts are obtained by neutralizing the acids with alkali, usually soda, either before or after the removal of the solvent by evaporation. I may incorporate with the sulfonic material other products having the nature of fillers, lubricants, binders or agglutinants and diluents to produce the consistency and the special qualities which may be desirable for any particular use.

As an example of a composition contemplated in my invention, the following is given:

No. 1.—150 parts amorphous graphite, 75 parts zinc dust; 60 parts sodium sulphonate, as described; 40 parts paraffin oil, 90 parts waste sulphite liquor, 10 parts water.

45 The paraffin oils may vary widely as to their properties but it is desirable for the oil to have a flash point sufficiently high to avoid danger of fire; oils with flash points from 150° F to 450° F are contemplated.

50 By waste sulphite liquor I refer to a waste

product in the manufacture of paper pulp by the sulphite process. This product is alkaline with glue-like properties and contains normally about 50% of water. The sulphite liquor may be evaporated to a sticky solid or semi-solid and may be used as such in my compositions, although in such case it would be better to add more water than if the sulphite liquor itself were used.

Other compounds are given as follows:

No. 2.—100 parts amorphous graphite, 50 parts sodium sulfonate, 50 parts paraffin oil.

No. 3—50 parts red lead, 85 parts amorphous graphite, 60 parts sodium sulfonate, 40 parts paraffin oil.

No. 4.—50 parts iron oxide, pulverized; 60 parts sodium sulfonate, 40 parts paraffin oil.

In the manufacture of my compositions, the sulfonate is dissolved in the oil in a heated condition and the waste sulphite, if used, is now added. The fillers may now be thoroughly incorporated by a mechanical mixer or otherwise and the mass may be thinned by addition of either water or oil.

My material is spread, smeared or brushed on the members of the joint before the union is effected and when applied to hot joints it expands and fills all tool marks and surface indentations, adhering strongly to the metal surfaces. Under heat and pressure the compound carbonizes, forming a firm, tight seal. As stated above, the joint may be easily broken and the metal surfaces are found clean and bright.

My compounds find application in sealing joints, in pipe lines carrying steam, ammonia and other gases, oils such as gasoline and lubricating oils, tar and the like. It is useful in making tight joints for oil well casings, hand holes, or man holes in boilers and stills including those operating at high temperatures and pressures, and may also be used as a coating for metallic or fiber gaskets. My invention is not to be limited by any theory as to the action of these compounds nor by any example, given by way of illustration, but only by the following claims.

I claim:

1. An improved sealing composition of the character described, comprising a filler, a

hydrocarbon oil and oil soluble sulfonate derived from hydrocarbon oil.

2. An improved hot joint composition comprising a pulverized mineral filler, paraffin oil and oil soluble sulfonate derived from hydrocarbon oil.

3. An improved hot joint composition comprising a pulverized mineral filler, paraffin oil, waste sulphite liquor and oil soluble sulfonate derived from hydrocarbon oil.

10 4. An improved hot joint composition capable of being thinned with either oil or water comprising a pulverized mineral filler, a paraffin oil, graphite and oil soluble sulfonate as described.

15 5. An improved hot joint composition capable of being thinned with either oil or water comprising a pulverized mineral filler, a paraffin oil, graphite and oil soluble sulfonate of an alkali metal.

20 6. An improved hot joint composition comprising 150 parts of amorphous graphite, 75 parts zinc dust, 40 parts paraffin oil, 90 parts waste sulphite liquor, 10 parts water, and 60 parts sodium sulfonate, as described.

25 In testimony that I claim the foregoing as my invention, I affix my signature.

JOSEPH C. WASSON.

30

35

40

45

50

55

60

65